

Oct. 5, 1926.

1,602,308

H. MALY

PROCESS OF SPINNING, DRAWING, AND DOUBLING YARN

Filed July 29, 1925 2. Sheets-Sheet 1



Inventor:  
Hermann Maly,  
By: Kneglit Bros,  
Attns.

Oct. 5, 1926.

1,602,308

H. MALY

PROCESS OF SPINNING, DRAWING, AND DOUBLING YARN

Filed July 29, 1925

2 Sheets-Sheet 2

Fig. 3.



Fig. 4.



Fig. 5.



Fig. 6.



Fig. 7.



Inventor:

Hermann Maly,  
By: Knight Bros.  
Atty.

Patented Oct. 5, 1926.

## UNITED STATES PATENT OFFICE.

HERMANN MALY, OF GUBEN, GERMANY.

## PROCESS OF SPINNING, DRAWING, AND DOUBLING YARN.

Application filed July 29, 1925, Serial No. 46,916, and in Germany August 1, 1924.

A usual practice in spinning yarn is to draw the rovings in a two-roller mule, and impart greater attenuation in a three-roller mule.

5 The object of my invention is to improve the uniformity, strength and fineness of the yarn and to insure that the twist is mainly at the circumferential part thereof; also to prevent back-twist, and secure greater tensile strength and stretchability.

10 In dealing with unspun rovings I attain these objects by disposing between the delivery rollers and the spindle, nearer to the former than to the latter, a brake or resistance 15 over which the fibre travels. Between this brake and the spindle the yarn is fully spun, and this longer portion of the yarn draws fibre from the loose bunch behind the brake, somewhat as occurred with the old distaff 20 and spindle. The brake effect is preferably made regulatable, so that the transmission of twist from the spun yarn to the loose fibre behind the brake can be regulated as required.

25 For doubling, the single yarns travel separately to the brake. The twist given for doubling is in the opposite direction to the twist of the fibres, so that there is some untwisting of the yarn, which allows of 30 stretching.

The invention is illustrated in the annexed drawings, which show various examples, Figs. 1 to 3 relating to spinning, and Figs. 4 to 7 to doubling.

35 As shown in Fig. 1 the delivery rollers  $a$ ,  $a'$  deliver loosely spun yarn  $b$ , which at  $c$  passes over a brake  $d$ , and thence to the spindle  $e$ . Owing to the provision of the brake, by far the greater part of the twist imparted 40 by the spindle is confined to that part of the yarn which is between the spindle and the brake. Between the spindle and brake there is little or no stretch, and the spun yarn draws out fibre in proportion as the speed of 45 the carriage exceeds the rate of delivery of the rollers.

The brake may be made vertically adjustable, for regulating its effect, or a larger or smaller brake may be substituted for the 50 same purpose; these two regulating methods may be used in conjunction. Fig. 1<sup>a</sup> shows a flat-topped brake across which the fibre runs from  $c$  to  $c'$ . I may also regulate the brake effect by vertically adjusting the 55 rollers, leaving the brake stationary.

For spinning and drawing yarn already partly spun the process is similar to that used for spinning from rovings, but the spindle  $e$  is rotated in the opposite direction to the twist of the partly spun yarn, with 60 such excess of speed that the part  $b$  leaving the rollers is untwisted.

For drawing and spinning with a three-roller mule, as shown in Fig. 3, the method is substantially the same, but about half the 65 drawing is preferably left to drawing rollers, the remaining half being effected by the combined spinning and drawing operation described.

With the apparatus shown in Fig. 5 for doubling, the brake  $d$  is so regulated, according to the yarn dealt with, that the untwisting effect due to rotating the spindle in the opposite direction to the twist of the 70 yarn does not proceed beyond the point  $c'$ , 75 or only does so to a predetermined, limited extent. The region of more or less loose fibre is in this case between  $c$  and  $c'$ . The yarns between  $c$  and  $b$  retain their original twist, and are not drawn. The yarn is 80 doubled at  $c'$ , or close to this point. There may be more than two yarns. By this method thread of good or fair strength may be obtained by doubling yarns where the 85 doubling and the twist of the yarns are in the same direction, or where the doubled yarns are of opposite twist, though with other methods such yarns are not at all strong.

The doubled yarn is in fact of a novel 90 kind. The doubling is permanent and independent of the direction of twist by which it is done, and of the twist of the separate 95 yarns. Irregularities of thickness of the separate yarns, such as shown at  $h$  in Fig. 4, are entirely eliminated in the doubled yarn, whereas with other methods they cause inequalities such as shown at  $g$  in Fig. 4.

Apart from the more thorough preparation of the rovings for the three-roller system, as compared with the two roller system, the spinning operations whereby the 100 yarns are formed are different with these two systems, as heretofore practised, but with my method yarns produced by the two-roller and three-roller systems are technically 105 yarns of the same kind, different only as regards the degree to which the fibres were prepared for spinning.

The distance between the rollers and 110

brake is made longer or shorter, according to the length of the fibres.

I have described the process with reference to mules, where the carriage with the 5 spindles is reciprocated, but I may employ it with system in which the spindles are stationary and the yarn feeders are on a carriage.

What I claim is:

10. 1. The method of spinning textile fibers, consisting in subjecting the fibers to a restraining influence adjacent the drawing or delivery rollers intermediate the latter and a mule spindle whereby the twist due to the rotation 15 of the spindle is imposed preponderantly on the length of fiber intermediate the point of application of said restraining influence and the spindle, the length of spun yarn drawing fiber from behind the point of application 20 of said restraining influence.
2. The method of spinning textile fibers, consisting in subjecting the fibers to a restraining influence adjacent the drawing or delivery rollers intermediate the latter and a mule 25 spindle whereby the twist due to the rotation of the spindle is imposed preponderantly on the length of fiber intermediate the point of application of said restraining influence and the spindle, the length of spun 30 yarn drawing fiber from behind the point of application of said restraining influence, and regulating the resistance of said restraining influence for controlling the transmission of twist from the spun yarn and the 35 fiber behind the point of application of said restraining influence.

3. The method of doubling yarn fibers, consisting in subjecting the yarn to a restraining influence adjacent the drawing or delivery rollers intermediate the latter and a mule spindle, and rotating the spindle in the opposite direction to the twist of the 40 yarn fibers whereby the separate yarns are untwisted between the rollers and the point of application of the restraining influence. 45

4. The method of doubling yarn fibers, consisting in subjecting the yarn to a restraining influence adjacent the drawing or delivery rollers intermediate the latter and a mule spindle, and rotating the spindle in 50 the opposite direction to the twist of the yarn fibers whereby the separate yarns are untwisted between the rollers and the point of application of the restraining influence, and adjusting the resistance of said restraining influence for controlling the longitudinal extent of the untwisting action. 55

5. The method of doubling yarn fibers, consisting in passing the separate yarns singly through drawing or delivery rollers, 60 subjecting the fibers to a restraining influence subsequent to their passage through the rollers, and winding the yarn on a spindle rotating in the opposite direction to the twist of the fibers, whereby the separate yarns are untwisted between the rollers and the point of application of the restraining influence and united substantially at said point. 65

In testimony whereof the foregoing specification is signed.

HERMANN MALY.